



US005769967A

# United States Patent [19]

## Dolan

[11] Patent Number: **5,769,967**  
[45] Date of Patent: **\*Jun. 23, 1998**

[54] **COMPOSITION AND PROCESS FOR TREATING METAL**

[75] Inventor: **Shawn E. Dolan**, Sterling Heights, Mich.

[73] Assignee: **Henkel Corporation**, Plymouth Meeting, Pa.

[\*] Notice: The term of this patent shall not extend beyond the expiration date of Pat. No. 5,281,282.

[21] Appl. No.: **674,558**

[22] Filed: **Jul. 2, 1996**

### Related U.S. Application Data

[63] Continuation of Ser. No. 429,431, Apr. 21, 1995, Pat. No. 5,534,082, which is a continuation-in-part of Ser. No. 213, 138, Mar. 15, 1994, abandoned, which is a continuation-in-part of Ser. No. 131,645, Oct. 5, 1993, Pat. No. 5,356,490, which is a continuation-in-part of Ser. No. 862,012, Apr. 1, 1992, Pat. No. 5,281,282.

[51] Int. Cl.<sup>6</sup> ..... **C23C 22/48**

[52] U.S. Cl. ..... **148/247; 140/268**

[58] Field of Search ..... 148/247, 268

[56] **References Cited**

### U.S. PATENT DOCUMENTS

2,276,353 3/1942 Thompson ..... 148/6

|           |         |                       |         |
|-----------|---------|-----------------------|---------|
| 2,507,956 | 5/1950  | Bruno et al. ....     | 148/6.2 |
| 2,796,370 | 6/1957  | Ostrander et al. .... | 148/6.2 |
| 2,796,371 | 6/1957  | Ostrander et al. .... | 148/6.2 |
| 2,798,829 | 7/1957  | Newhard et al. ....   | 148/6.2 |
| 2,825,697 | 3/1958  | Carroll et al. ....   | 252/389 |
| 4,370,173 | 1/1983  | Dollman ....          | 134/3   |
| 4,762,638 | 8/1988  | Dollman et al. ....   | 252/135 |
| 4,963,596 | 10/1990 | Lindert et al. ....   | 526/313 |
| 5,281,282 | 1/1994  | Dolan et al. ....     | 148/247 |

Primary Examiner—Sam Silverberg

Attorney, Agent, or Firm—Ernest G. Szoke; Wayne C. Jaeschke; Norvell E. Wisdom, Jr.

[57] **ABSTRACT**

Heating an aqueous mixture of a fluoroacid such as  $H_2TiF_6$  and an oxide, hydroxide, and/or carbonate such as silica produces a clear mixture with long term stability against settling of any solid phase, even when the oxide, hydroxide, or carbonate phase before heating was a dispersed solid with sufficiently large particles to scatter light and make the mixture before heating cloudy. The clear mixture produced by heating can be mixed with soluble hexavalent and/or trivalent chromium, and preferably also nitrate and chloride ions to produce a composition that provides a conversion coating with good protection against corrosion while requiring substantially less chromium than previous coatings of equal corrosion protective quality.

**19 Claims, No Drawings**

## 1

COMPOSITION AND PROCESS FOR  
TREATING METALCROSS-REFERENCE TO RELATED  
APPLICATIONS

This application is a continuation of application Ser. No. 429,431 filed Apr. 21, 1995, now U.S. Pat. No. 5,534,082, which was a continuation-in-part of Ser. No. 213,138 of Mar. 15, 1994, now abandoned, which was a continuation-in-part of Ser. No. 131,645 of Oct. 5, 1993, now U.S. Pat. No. 5,356,490, which was a continuation-in-part of Ser. No. 862,012 of Apr. 1, 1992, now U.S. Pat. No. 5,281,282.

## BACKGROUND OF THE INVENTION

## 1. Field of the Invention

This invention relates to processes of treating metal surfaces with aqueous acidic compositions to increase the resistance to corrosion of the treated metal surface, either as thus treated or after subsequent overcoating with some conventional organic based protective layer. A major object of the invention is to provide a storage stable, preferably single package, treatment that can be substantially free from hexavalent chromium but can protect metals substantially as well as the hexavalent chromium containing treatments of the prior art, or can improve the stability of treatment solutions that do contain hexavalent chromium and/or reduce the amount of chromium needed with such solutions to provide a specified degree of corrosion protection. This invention also relates to reaction of fluorometallic acids with other metal or metalloid containing materials to produce compositions or intermediates for compositions useful for such treatments.

## 2. Statement of Related Art

A very wide variety of materials have been taught in the prior art for the general purposes of the present invention, but most of them contain hexavalent chromium or other inorganic oxidizing agents which are environmentally undesirable. Also, many of the prior art treatment compositions include components that are chemically or physically unstable when mixed, so that single package concentrates for such treatment compositions are not practical.

## DESCRIPTION OF THE INVENTION

## GENERAL PRINCIPLES OF DESCRIPTION

Except in the claims and the operating examples, or where otherwise expressly indicated, all numerical quantities in this description indicating amounts of material or conditions of reaction and/or use are to be understood as modified by the word "about" in describing the broadest scope of the invention. Practice within the numerical limits stated is generally preferred, however. Also in this description, unless expressly stated to the contrary: percent, "parts of", and ratio values are by weight; the term "polymer" includes "oligomer", "copolymer", "terpolymer", and the like; the description of a group or class of materials as suitable or preferred for a given purpose in connection with the invention implies that mixtures of any two or more of the members of the group or class are equally suitable or preferred; description of constituents in chemical terms refers to the constituents at the time of addition to any combination specified in the description, and does not necessarily preclude chemical interactions among the constituents of a mixture once mixed; specification of materials in ionic form implies the presence of sufficient counterions to

## 2

produce electrical neutrality for the composition as a whole (any counterions thus implicitly specified should preferably be selected from among other constituents explicitly specified in ionic form, to the extent possible; otherwise such counterions may be freely selected, except for avoiding counterions that act adversely to the stated objects of the invention); and the term "mole" and its variations may be applied to elemental, ionic, and any other chemical species defined by number and type of atoms present, as well as to 10 compounds with well defined molecules.

## OBJECTS OF THE INVENTION

Various alternative or concurrent objects of the invention include: providing better corrosion resistance at no more 15 than equal cost or equal corrosion resistance at lower cost to metal surfaces, particularly those of aluminum; reducing the amount of chromium and/or other polluting chemicals needed to provide a specified degree of corrosion protection; and improving the adherence of paint and like materials to 20 metal surfaces treated according to the invention. Other objects will be apparent from the description below.

## SUMMARY OF THE INVENTION

It has been found that aqueous compositions comprising 25 (A) a component of dissolved fluoroacids of one or more metals and metalloid elements selected from the group of elements consisting of titanium, zirconium, hafnium, boron, aluminum, silicon, germanium, and tin and, (B) a component of one or more of (i) dissolved or dispersed finely 30 divided forms of metals and metalloid elements selected from the group of elements consisting of titanium, zirconium, hafnium, boron, aluminum, silicon, germanium, and tin and (ii) the oxides, hydroxides, and carbonates of 35 such metals and metalloid elements can be caused to chemically interact in such a manner as to produce a composition useful for novel metal treatments. If component (B) is present in dispersion rather than solution, as is generally preferred, the initial composition normally will not be optically transparent, because of the scattering of visible light, in a thickness of 1 centimeter ("cm"), and the occurrence of the 40 desired chemical interaction can be determined by the clarification of the composition. If components (A) and (B) as defined above are both present in the precursor aqueous composition in sufficiently high concentrations, adequate 45 chemical interaction between them may occur at normal ambient temperatures (i.e., 20°-25° C.) within a practical reaction time of 24 hours or less, particularly if component (B) is dissolved or dispersed in very finely divided form. 50 Mechanical agitation may be useful in speeding the desired chemical interaction and if so is preferably used. Heating, even to relatively low temperatures such as 30° C., is often useful in speeding the desired chemical interaction, and if it does so speed the reaction is usually preferred. The desired 55 chemical interaction between components (A) and (B) of the mixed composition eliminates or at least markedly reduces any tendency toward settling of a dispersed phase that might otherwise occur upon long term storage of the initial mixture of components (A) and (B) as defined above.

The compositions resulting from chemical interaction as 60 described above may then be utilized as metal treating compositions, optionally after being combined with a component (C) that is either (i) a water soluble or dispersible polymer and/or copolymer, preferably selected from the group consisting of (i. 1) polymers and copolymers of one or more x-(N—R<sup>1</sup>—N—R<sup>2</sup>-aminomethyl)-4-hydroxy-65 styrenes, where x=2, 4, 5, or 6, R<sup>1</sup> represents an alkyl group

containing from 1 to 4 carbon atoms, preferably a methyl group, and  $R^2$  represents a substituent group conforming to the general formula  $H(CHOH)_nCH_2-$ , where  $n$  is an integer from 1 to 7, preferably from 3 to 5, (i.2) epoxy resins, particularly polymers of the diglycidylether of bisphenol-A, optionally capped on the ends with non-polymerizable groups and/or having some of the epoxy groups hydrolyzed to hydroxyl groups, and (i.3) polymers and copolymers of acrylic and methacrylic acids and their salts; or (ii) a composition containing hexavalent chromium, and, optionally, trivalent chromium.

Optionally, another component (D) made up of water soluble oxides, carbonates, or hydroxides of at least one of Ti, Zr, Hf, B, Al, Si, Ge, and Sn may also be added before, after, or simultaneously with component (C) but after the interaction of components (A) and (B). For this purpose, "water soluble" means a solubility to at least 1% in water at normal ambient temperature, and "water insoluble" means less soluble than this.

The resulting compositions are suitable for treating metal surfaces to achieve excellent resistance to corrosion, particularly after subsequent conventional coating with an organic binder containing protective coating. The compositions are particularly useful on iron and steel, galvanized iron and steel, zinc and those of its alloys that contain at least 50 atomic percent zinc, and, most preferably, aluminum and its alloys that contain at least 50 atomic percent aluminum. The treating may consist either of coating the metal with a liquid film of the composition and then drying this liquid film in place on the surface of the metal, or simply contacting the metal with the composition for a sufficient time to produce an improvement in the resistance of the surface to corrosion, and subsequently rinsing before drying. Such contact may be achieved by spraying, immersion, and the like as known per se in the art. When immersion is used, it is optional, and often advantageous, to contact the metal surface with an aqueous composition comprising polymers and copolymers of one or more  $x$ -( $N-R^1-N-R^2$ -aminomethyl)-4-hydroxy-styrenes, where  $x=2, 4, 5$ , or 6,  $R^1$  represents an alkyl group containing from 1 to 4 carbon atoms, preferably a methyl group, and  $R^2$  represents a substituent group conforming to the general formula  $H(CHOH)_nCH_2-$ , where  $n$  is an integer from 1 to 7, preferably from 3 to 5, after contacting the metal with a composition containing components (A) and (B) as described above, removing the metal from contact with this composition containing components (A) and (B) as described above, and rinsing with water, but before drying.

The invention also provides a process for effectively coating the above-stated metallic surfaces in the absence of an intermediate rinsing step. The process comprises the steps of (i) cleaning the metal surface to be coated, (ii) rinsing the cleaned metal surface with water so as to remove any excess cleaning solution, (iii) contacting the metallic surface with the above-described coating composition, and (iv) drying the coated metallic surface.

There is also another embodiment of the present invention which provides a composition and process for coating surfaces of aluminum and alloys thereof, wherein the composition comprises, preferably consists essentially of, or more preferably consists of, water and a mixture of: (A') a water soluble or dispersible polymer having at least one alcohol functionality selected from the group consisting of polyvinyl alcohol, polyethylene glycol, modified starch, and mixtures thereof and (B') polymers and copolymers of acrylic and methacrylic acid and their salts, and, optionally, one or more of the following: a component (C') selected

from the group consisting of the same fluorometallic acids, with the same preferences, as recited for component (A) herein; a component (D') of the same metallic and/or metalloid elements and their oxides, hydroxides, and/or carbonates, with the same preferences, as recited for component (B) herein; and a component (E') selected from the group consisting of the same water soluble oxides, carbonates, or hydroxides of at least one of Ti, Zr, Hf, B, Al, Si, Ge, and Sn, with the same preferences, as recited for component (D) herein.

It should be understood, as already pointed out above, that the descriptions of compositions above do not preclude the possibility of unspecified chemical interactions among the components listed, but instead describes the components of a composition according to the invention in the form in which they are generally used as ingredients to prepare such a composition. In fact, a chemical interaction, most probably to produce oxyfluoro complexes of the metal or metalloid elements or their compounds heated in contact with fluorometallic acids, is believed to occur, but the invention is not limited by any such theory.

#### DESCRIPTION OF PREFERRED EMBODIMENTS

To the extent that their water solubility is sufficient, the fluoroacid component (A) to be caused to interact in a mixture with water and one or more metals and/or metalloid elements and/or oxides, hydroxides, and/or carbonates thereof in a process according to one embodiment of the invention may be freely selected from the group consisting of  $H_2TiF_6$ ,  $H_2ZrF_6$ ,  $H_2HfF_6$ ,  $H_3AlF_6$ ,  $H_2SiF_6$ ,  $H_2GeF_6$ ,  $H_2SnF_6$ ,  $HBF_4$ , and mixtures thereof.  $H_2TiF_6$ ,  $H_2ZrF_6$ ,  $H_2HfF_6$ ,  $H_2SiF_6$ ,  $HBF_4$ , and mixtures thereof are preferred;  $H_2TiF_6$ ,  $H_2ZrF_6$ ,  $H_2SiF_6$  and mixtures thereof are more preferred; and  $H_2TiF_6$  is most preferred. The concentration of fluoroacid component at the time of interaction preferably is at least, with increasing preference in the order given, 0.01, 0.02, 0.04, 0.08, 0.12, 0.16, 0.20, 0.24, 0.27, 0.29, 0.31, 0.33, 0.35, 0.360, 0.365, 0.370, 0.375, 0.380, or 0.385 moles per kilogram (hereinafter usually abbreviated as "M/kg") of the total mixture in which the interaction with component (B) occurs and independently preferably is not more than, with increasing preference in the order given, 7, 5, 3, 2.0, 1.5, 1.0, 0.80, 0.65, 0.60, 0.55, 0.50, 0.45, 0.42, or 0.40 M/kg of the total mixture in which the interaction with component (B) occurs.

Component (B) of metallic and/or metalloid elements and/or their oxides, hydroxides, and/or carbonates is preferably selected from the group consisting of the oxides, hydroxides, and/or carbonates of silicon, zirconium, and/or aluminum, more preferably includes silica, and still more preferably includes both zirconium and silicon in a molar ratio of silicon to zirconium that is at least, with increasing preference in the order given, 0.5:1.0, 0.7:1.0, 0.9:1.0, 1.1:1.0, 1.20:1.0, 1.30:1.0, 1.40:1.0, 1.45:1.0, 1.50:1.0, 1.55:1.0, 1.60:1.0, 1.65:1.0, 1.70:1.0, 1.75:1.0, 1.79:1.0, or 1.83:1.0 and independently preferably is not more than, with increasing preference in the order given, 7:1.0, 5:1.0, 4.0:1.0, 3.5:1.0, 3.0:1.0, 2.7:1.0, 2.5:1.0, 2.3:1.0, 2.1:1.0, or 1.9:1.0.

Any form of component (B) that is sufficiently finely divided to be readily dispersed in water may be used in a process according to one embodiment of this invention, but for constituents of this component that have low solubility in water it is preferred that the constituent be amorphous rather than crystalline, because crystalline constituents can require

a much longer period of heating and/or a higher temperature of heating to produce a composition that is no longer susceptible to settling and optically transparent. Solutions and/or sols such as silicic acid sols may be used, but, if the composition according to the invention that is made with them is intended for use by drying a layer of it into place on a surface to be treated, it is highly preferable, as described further below, that the solutions and/or sols be substantially free from alkali metal ions. However, it is generally most preferred to use dispersions of very finely divided silica made by pyrogenic processes.

The ratio of total moles of fluoroacid component (A) to total moles of component (B) in an aqueous composition heated according to one embodiment of this invention preferably is from 1:1 to 50:1, more preferably from 1.5:1.0 to 20:1, or still more preferably from 1.5:1 to 5.0:1.0, except that if component (B) includes both silicon and zirconium and the composition made is ultimately intended to contain hexavalent chromium, the ratio of total moles of fluoroacid component (A) to total moles of component (B) instead preferably is at least, with increasing preference in the order given, 0.05:1.0, 0.10:1.0, 0.20:1.0, 0.30:1.0, 0.40:1.0, 0.50:1.0, 0.55:1.0, 0.60:1.0, 0.65:1.0, 0.70:1.0, 0.75:1.0, 0.80:1.0, or 0.85:1.0 and independently preferably is not more than, with increasing preference in the order given, 5.0:1.0, 4.0:1.0, 3.0:1.0, 2.5:1.0, 2.0:1.0, 1.5:1.0, 1.2:1.0, 1.0:1.0, or 0.90:1.0.

According to one embodiment of the invention, an aqueous liquid composition comprising, preferably consisting essentially of, or more preferably consisting of, water and components (A) and (B) as described above, which composition (i) scatters visible light, (ii) is not optically transparent in a thickness of 1 cm, and/or (iii) undergoes an extent of settling of a solid phase that is detectable with unaided human vision if maintained for at least 100 hours at a temperature between its freezing point and 20° C., is maintained at a temperature of at least 21° C., optionally with mechanical agitation, for a sufficient time to produce a composition that (i) does not suffer any visually detectable settling when stored for a period of 100, or more preferably 1000, hours and (ii) is optically transparent in a thickness of 1 cm. Preferably, the temperature at which the initial mixture of components (A) and (B) is maintained is in the range from 25° to 100° C., or more preferably within the range from 30° to 80° C., and the time that the composition is maintained within the stated temperature range is within the range from 3 to 480, more preferably from 5 to 90, or still more preferably from 10 to 30, minutes (hereinafter often abbreviated "min"). Shorter times and lower temperatures within these ranges are generally adequate for converting compositions in which the component (B) is selected only from dissolved species and/or dispersed amorphous species without any surface treatment to reduce their hydrophilicity, while longer times and/or higher temperatures within these ranges are likely to be needed if component (B) includes dispersed solid crystalline materials and/or solids with surfaces treated to reduce their hydrophilicity. With suitable equipment for pressurizing the reaction mixture, even higher temperatures than 100° C. can be used in especially difficult cases.

Independently, it is preferred that the pH of the aqueous liquid composition combining components (A) and (B) as described above be kept in the range from 0 to 4, more preferably in the range from 0.0 to 2.0, or still more preferably in the range from 0.0 to 1.0 before beginning maintenance at a temperature of at least 21° C. as described above.

A composition made as described immediately above is suitable for use as a protective treatment for metals. In many cases, however, a better protective treatment composition may be obtained by mixing the product of interaction between components (A) and (B) as described above with a third component (C) as also noted above. To make such compositions including component (C), after maintenance of a composition containing components (A) and (B) as described above at a temperature and for a time sufficient to promote their interaction, the composition is preferably brought if necessary to a temperature below 30° C. and then mixed with a component consisting of at least one of (i) at least one water soluble or dispersible polymer and/or copolymer, preferably selected from the group consisting of (i.1) polyhydroxyl alkylamino derivatives of poly{p-hydroxystyrene} as described above and, in more detail, in U.S. Pat. No. 4,963,596, the entire disclosure of which, except to the extent contrary to any explicit statement herein, is hereby incorporated herein by reference, (i.2) epoxy resins, particularly polymers of the diglycidylether of bisphenol-A, optionally capped on the ends with non-polymerizable groups and/or having some of the epoxy groups hydrolyzed to hydroxyl groups, and (i.3) polymers and copolymers of acrylic and methacrylic acids and their salts; and (ii) a composition containing hexavalent chromium, and, optionally, trivalent chromium, as known per se in the art for treating metals, particularly aluminum and its alloys, to retard corrosion thereon. Suitable and preferred water soluble polymers and methods of preparing them are described in detail in U.S. Pat. No. 4,963,596. Preferably, the ratio by weight of the solids content of component (C) to the total of active ingredients of component (A) as described above is in the range from 0.1 to 3, more preferably from 0.2 to 2, or still more preferably from 0.20 to 1.6, except that when component (C) is predominantly constituted of compounds of hexavalent chromium, the molar ratio of chromium atoms in component (C) to the total of metal and metalloid atoms in components (A) and (B) preferably is at least, with increasing preference in the order given, 0.3:1.0, 0.5:1.0, 0.7:1.0, 0.80:1.0, 0.90:1.0, 0.95:1.0, 1.00:1.0, 1.05:1.0, or 1.10:1.0 and independently preferably is not more than, with increasing preference in the order given, 10:1.0, 8:1.0, 6:1.0, 4.0:1.0, 3.0:1.0, 2.7:1.0, 2.4:1.0, 2.1:1.0, 1.9:1.0, 1.7:1.0, 1.5:1.0, 1.40:1.0, 1.35:1.0, 1.30:1.0, 1.25:1.0, 1.20:1.0, or 1.15:1.0.

The preferred concentration of components (A) and (B) in a working composition according to the invention that includes hexavalent chromium compounds as a predominant part of component (C) is considerably less than the concentrations specified above as preferred for the initial interaction between components (A) and (B). Specifically, in a working composition according to the invention, suitable for direct contact with a metal substrate to form a corrosion resistant coating thereon, the total concentration of titanium, zirconium, hafnium, boron, aluminum, silicon, germanium, and tin atoms from component (A) preferably is at least, with increasing preference in the order given, 1.0, 2.0, 4.0, 6.0, 8.0, 10, 12, 14, 16, 18, or 19 millimoles per liter (hereinafter usually abbreviated as "mM/L") and independently preferably is not more than, with increasing preference in the order given, 200, 150, 100, 80, 60, 50, 40, 35, 30, 25, or 21 mM/L. Concentrations of other constituents of working compositions preferably are such as to result in ratios to the concentration of component (A) and to one another as already specified above.

A composition prepared by a process as described above constitutes another embodiment of this invention. It is

normally preferred that compositions according to the invention as defined above should be substantially free from many ingredients used in compositions for similar purposes in the prior art. Specifically, it is often increasingly preferred in the order given, independently for each preferably minimized component listed below, that these compositions, when directly contacted with metal in a process according to this invention, contain no more than 1.0, 0.35, 0.10, 0.08, 0.04, 0.02, 0.01, or 0.001% of each of the following constituents: hexavalent chromium; ferricyanide; ferrocyanide; anions containing molybdenum or tungsten; nitrates and other oxidizing agents (the others being measured as their oxidizing stoichiometric equivalent as nitrate); phosphorus and sulfur containing anions that are not oxidizing agents; alkali metal and ammonium cations; and organic compounds with two or more hydroxyl groups per molecule and a molecular weight of less than 300, except that:

- (i) the preference for minimal amounts of alkali metal and ammonium cations applies only to compositions used for processes according to the invention that include drying into place on the metal surface to be treated without rinsing after contact between the metal surface and the composition containing at least components (A) and (B) as described above; when a composition according to the invention is contacted with a metal surface and the metal surface is subsequently rinsed with water before being dried, any alkali metal and ammonium ions present are usually removed by the rinsing to a sufficient degree to avoid any substantial diminution of the protective value of subsequently applied organic binder containing protective coatings;
- (ii) the preference for minimization of the amount of hexavalent chromium present is due to the polluting effect of hexavalent chromium, and where there is an absence of legal restraints against pollution and/or sufficiently economical means of disposing of the hexavalent chromium without environmental damage exist, this preference does not apply; in fact, in one specialized embodiment of the invention, as already noted above, hexavalent chromium may advantageously be incorporated into working compositions according to this invention themselves, and in another specialized embodiment of the invention, liquid compositions containing hexavalent chromium may be used as posttreatments after application of a coating according to this invention but before final overcoating with a paint or the like, in order further to improve corrosion resistance of the metal surface treated; and
- (iii) if substantial amounts of hexavalent chromium are present in compositions according to the invention, the preference against nitrates and other oxidizing agents does not apply; in fact, in such compositions it is normally preferred, in order to obtain coatings with sufficient corrosion protective value in shorter times and/or at lower temperatures, for a working composition according to the invention to contain another oxidizing component, often designated for convenience hereinafter as optional component (E), that comprises, preferably consists essentially of, or more preferably consists of oxidizing agents other than compounds containing hexavalent chromium.

Independently, when it is present, component (E) preferably comprises both (E. 1) nitrate ions and (E.2) halide ions. In a working composition according to the invention, the concentration of nitrate ions when present independently preferably is at least, with increasing preference in the order given, 1, 2, 4, 6, 8, 10, 12, 14, or 16 mM/L and indepen-

dently preferably is not more than, with increasing preference in the order given, 100, 75, 50, 40, 30, 26, 23, 21, 19, or 18 mM/L. Also, the concentration of halide ions when present independently preferably is at least, with increasing preference in the order given, 0.01, 0.02, 0.04, 0.08, 0.15, 0.20, 0.30, 0.35, 0.40, 0.45, or 0.50 mM/L and independently preferably is not more than, with increasing preference in the order given, 50, 30, 20, 10, 5, 4.0, 3.0, 2.0, 1.0, 0.80, 0.70, 0.65, 0.60, or 0.55 mM/L. Any fluoride ions that might be present in the composition as a result of dissociation of part of component (A) are not to be considered as halide ions for the purpose of measuring these preferred concentrations; instead, only separately added salts or acids containing and/or dissociating to uncomplexed halide ions are to be considered. Both nitrate ions and halide ions are preferably supplied to the composition by addition of water soluble salts containing these ions; primarily for reasons of economy, these salts are preferably alkali metal salts, most preferably sodium salts. Independently, the halide ions for optional component (E.2), primarily for reasons of economy, are preferably chloride ions.

The other major type of coating used in the invention, employing a coating composition including necessary components (A') and (B') as already described above, has been found to be especially useful for treating metallic surfaces that are exposed to alkali metal ions, particularly sodium such as often occurs in detergents and other cleaners, after the treatment with a composition according to this invention has been completed. (Protective coatings applied to metallic surfaces, particularly aluminum, preferably are water insoluble and inhibit corrosion. However, metallic surfaces bearing a protective coating are often exposed to sodium ions later. It is believed that, upon exposure of some prior art coatings to sodium ions, the sodium ions oftentimes at least partially replace the aluminum in the formed coating, much as in an ion-exchange resin; such replacement in turn causes the film coating to be water sensitive, by increasing its solubility in water.) In an effort to decrease adverse effects of alkali metal ions on the treated surfaces, it has been found that by combining (i) polymers and copolymers of acrylic and methacrylic acids and their salts having an average molecular weight of about 50,000 with (ii) a water soluble or dispersible polymer having at least one —OH group per polymer molecule, adverse effects from exposure of the treated surface to alkali metal ions can be reduced. Possibly this occurs because the alcohol functionality cross-links by esterification with the acid functions. In a particularly preferred embodiment of this embodiment of the invention, the composition contacted with a metallic surface comprises, preferably consists essentially of, or more preferably consists of water and: (A') from 0.5 to 50 g/l and (B') from 0.5 to 50, and more preferably from 0.5 to 16 g/l of polyvinyl alcohol. The polyvinyl alcohol used in the invention preferably is a low molecular weight polyvinyl alcohol which is 75–99+mole % hydrolyzed, and has an average degree of polymerization ranging from 100–600.

While any water soluble or dispersible polymer having at least one —OH group per polymer molecule may be employed without departing from the spirit of this embodiment of the invention, preferred polymers and amounts thereof include the above-stated polyvinyl alcohol; from 0.3 to 16 g/l, preferably from 0.3 to 1.2 g/l, of polyethylene glycol having a molecular weight of from 90,000 to 900,000; and from 0.5 to 16 g/l, preferably from 0.5 to 10 g/l of dextrin, cyclodextrin, or a modified starch.

The term "modified starch" is one commonly known in the art. It refers to any of several water-soluble polymers

derived from a starch by acetylation, chlorination, acid hydrolysis, or enzymatic action. These reactions yield starch acetates, esters, and ethers in the form of stable and fluid solutions and films. These starch derivatives useful herein are well known.

The hydroxalkyl starch ethers and starch esters can be obtained by known etherification and esterification processes. These starch ethers and esters should have a degree of substitution (hereinafter often abbreviated "D.S.") of 0.01 to 0.5, and preferably 0.1 to 0.5. As used herein D.S. means the average degree of substitution, per anhydroglucose unit of the corresponding unmodified starch, of hydroxyl groups in the starch by chemical modifying substituents, such as, for example, hydroxalkyl and/or carbonyl groups.

Oxidized starch can be obtained by known processes involving oxidation of starch with a suitable oxidizing agent, as for example sodium hypochlorite, potassium dichromate and sodium permanganate. The starch can be oxidized under acidic, alkaline or neutral conditions, and the resulting product can contain carboxyl and carbonyl groups. Preferably the oxidized starch has a "D.O." value of 0.01 to 1.0, where "D.O." refers to the number of carboxyl groups introduced per anhydroglucose unit of the corresponding unmodified starch. These starch derivatives and methods for obtaining them are discussed in Whistler and Paschall (eds.), *Starch: Chemistry and Technology*, vol. I, (Academic Press, New York, 1965), pp. 458-78.

Dextrins and cyclodextrins are polysaccharide products of a complex nature resulting from the partial degradation of starch, such as corn starch, potato starch, wheat starch, and the like, with heat, as for example, by roasting with acid or alkaline catalysts. Linear and branched dextrins are classified in three types. The particular type obtained depends on the heating time, temperature, and catalyst employed in the treatment of the starch. These types are classified as white dextrins, yellow or canary dextrins, and British gums, and all such dextrins are suitable herein. White and canary dextrins are preferred because British gums are brown in color. White dextrins are preferably pregelatinized (made water soluble during manufacture), if necessary, to render them more readily mixed with other water soluble components. Dextrins and methods for obtaining them are well known. See, for example, Whistler and Paschall, *op. cit.*, vol. I, p. 421 ff and vol. II, p. 253 ff.

The starch hydrolysates useful in the compositions of this invention are a relatively new class of starch materials. These starch hydrolysates are made by subjecting a source of starch, such as hereinbefore mentioned, to enzyme or acid treatment or a combination of both. It is important that the starch hydrolysate have a relatively low dextrose equivalent (hereinafter often abbreviated "D.E."). The starch hydrolysate should have a D.E. of from 2 to 35, and preferably have a D.E. of from 5 to 25. The most preferred materials have a D.E. within the range of 5 to 15. (The term D.E. is used herein to refer to the reducing sugars content of the dissolved solids in a starch hydrolysate expressed as percent dextrose as measured by the Luff-Schoorl method [NBS Circular C-40, p. 195; also appearing in *Polarimetry, Saccharimet, and the Sugars* published by Frederick J. Bates and Associates].)

Particularly preferred modified starches include cyclodextrins, which are macro-cyclic non-reducing D-glucosyl polymers containing six or more D-glucosyl residues bonded by  $\alpha$ -(1,4) links. A more detailed description of cyclodextrins can be found in Whistler and Paschall, *op. cit.*, Vol. 1, pp. 209-224.

The pH of a composition according to this invention that contains components (A') and (B') as necessary components

preferably is in the range from 1.0 to 5.0, and more preferably from 1.0 to 3.5.

In a preferred embodiment of the aspect of the invention utilizing necessary components (A') and (B'), the treating composition also includes from 0.2 to 19.0, and more preferably from 0.2 to 8.0 g/l, of fluoroacids component (C') admixed therein. Component (C') is preferably selected from the group consisting of  $H_2TiF_6$ ,  $H_2ZrF_6$ , and  $H_2SiF_6$ , and more preferably is  $H_2TiF_6$  or  $H_2ZrF_6$ .

Still another embodiment of the invention is a process of treating a metal with a composition prepared as described above. In one embodiment of the invention, it is preferred that the aqueous composition as described above be applied to the metal surface and dried in place thereon. For example, 15 coating the metal with a liquid film may be accomplished by immersing the surface in a container of the liquid composition, spraying the composition on the surface, coating the surface by passing it between upper and lower rollers with the lower roller immersed in a container of the liquid composition, and the like, or by a mixture of methods. 20 Excessive amounts of the liquid composition that might otherwise remain on the surface prior to drying may be removed before drying by any convenient method, such as drainage under the influence of gravity, squeegees, passing between rolls spaced a short specified distance apart, and the like.

If the surface to be coated is a continuous flat sheet or coil and precisely controllable coating techniques such as gravure roll coaters are used, a relatively small volume per unit 30 area of a concentrated composition may effectively be used for direct application. On the other hand, if the coating equipment used does not readily permit precise coating at low coating add-on liquid volume levels, it is equally effective to use a more dilute acidic aqueous composition to 35 apply a thicker liquid coating that contains the same amount of active ingredients. In either case, when compositions according to the invention containing necessary ingredients (A) and (B) as described above are used, it is preferred that the total amount of active ingredients of components (A), 40 (B), and (C) as described above that are dried into place on the surface to be treated, or that remain as add-on mass on the surface after exposure to a working composition according to the invention and subsequent rinsing and, optionally, 45 drying, is at least, with increasing preference in the order given, 1, 2, 4, 8, 15, 30, 50, 70, 80, 90, 100, 110, 120, or 125 milligrams per square meter (hereinafter often abbreviated as "mg/m<sup>2</sup>") of surface area treated and independently, primarily for reasons of economy, preferably is not more than 500, 400, 300, 250, 200, 180, 170, 150, or 140 mg/m<sup>2</sup>.

Drying may be accomplished by any convenient method, of which many are known per se in the art; examples are hot air and infrared radiative drying. Independently, it is preferred that the maximum temperature of the metal reached during drying fall within the range from 30 to 200, more 55 preferably from 30 to 150, still more preferably from 30 to 75, °C. Also independently, it is often preferred that the drying be completed within a time ranging from 0.5 to 300, more preferably from 2 to 50, still more preferably from 2 to 10, seconds (hereinafter abbreviated "sec") after coating 60 is completed.

According to an alternative embodiment of the invention, the metal to be treated preferably is contacted with a composition prepared as described above at a temperature that is at least, with increasing preference in the order given, 65 15°, 18°, 21°, 24°, or 26° C. and independently, primarily for reasons of economy, preferably is not more than, with increasing preference in the order given, 90°, 85°, 80°, 70°,

## 11

65°, or 60° C. and if the composition contains hexavalent chromium compounds as the predominant part of component (C), still more preferably is not more than, with increasing preference in the order given, 55°, 50°, 45°, 40°, 35°, 32°, or 29° C. Independently, the metal to be treated preferably remains in contact with a working composition according to the invention for a time that is at least, with increasing preference in the order given, 1, 3, 5, 7, 9, 20, or 30 sec and, if the working composition according to the invention contains a component (C) that is constituted predominantly of compounds containing hexavalent chromium more preferably is at least, with increasing preference in the order given, 50, 75, 100, 125, 150, or 175 sec and independently, primarily for reasons of economy, preferably is not more than, with increasing preference in the order given, 1800, 1200, 600, or 300 sec and unless the working composition according to the invention contains a component (C) that is constituted predominantly of compounds containing hexavalent chromium more preferably is not more than, with increasing preference in the order given, 200, 100, 75, 50, or 30 sec, and the metal surface thus treated is subsequently rinsed with water in one or more stages before being dried. In this embodiment, at least one rinse, preferably the last rinse, after treatment with a composition according to this invention preferably is with deionized, distilled, or otherwise purified water. Also in this embodiment, it is preferred that the maximum temperature of the metal reached during drying fall within the range from 30 to 200, more preferably from 30 to 150, or still more preferably from 30 to 75, °C. and that, independently, drying be completed within a time ranging from 0.5 to 300, more preferably from 2 to 50, still more preferably from 2 to 10, sec after the last contact of the treated metal with a liquid before drying is completed.

A process according to the invention as generally described in its essential features above may be, and usually preferably is, continued by coating the dried metal surface produced by the treatment as described above with a siccative coating or other protective coating, relatively thick as compared with the coating formed by the earlier stages of a process according to the invention as described above. Such protective coatings may generally, in connection with this invention, be selected and applied as known per se in the art. Surfaces thus coated have been found to have excellent resistance to subsequent corrosion, as illustrated in the examples below. Particularly preferred types of protective coatings for use in conjunction with this invention include acrylic and polyester based paints, enamels, lacquers, and the like. However, in the specialized embodiment of the invention described above wherein the working composition according to the invention contains a component (C) that is constituted predominantly of compounds containing hexavalent chromium, excellent corrosion resistance, particularly on aluminum, can be achieved even without subsequently covering a surface treated with a composition according to the invention with any such additional protective coating.

In a process according to the invention that includes other steps after the formation of a protective layer on the surface of a metal by contacting the metal with a composition according to the invention as described above and that operates in an environment in which the discharge of hexavalent chromium is either legally restricted or economically handicapped, it is generally preferred that none of these other steps include contacting the surfaces with any composition that contains more than, with increasing preference in the order given, 1.0, 0.35, 0.10, 0.08, 0.04, 0.02, 0.01,

## 12

0.003, 0.001, or 0.0002% of hexavalent chromium. Examples of suitable and preferred chromium free treatments are described in U.S. Pat. No. 4,963,596. However, in certain specialized instances, hexavalent chromium may 5 impart sufficient additional corrosion protection to the treated metal surfaces to justify the increased cost of using and lawfully disposing of it.

Preferably, the metal surface to be treated according to the invention is first cleaned of any contaminants, particularly 10 organic contaminants and foreign metal fines and/or inclusions. Such cleaning may be accomplished by methods known to those skilled in the art and adapted to the particular type of metal substrate to be treated. For example, for galvanized steel surfaces, the substrate is most preferably cleaned with a conventional hot alkaline cleaner, then rinsed with hot water, squeegeed, and dried. For aluminum, the surface to be treated most preferably is first contacted with 15 either an aqueous alkaline cleaning solution in accordance with that disclosed in U.S. Pat. No. 4,762,638, incorporated herein by reference, or an aqueous acidic cleaning solution as disclosed in U.S. Pat. No. 4,370,173, also incorporated herein by reference. With respect to the aqueous acidic cleaning solution, it should also be noted that a source of fluoride such as HF may also be employed to even further 20 enhance the cleaning process. Irrespective of the type of cleaning solution employed, the aluminum is then subjected to a water rinse and optionally but preferably to a deoxidizing process as known in the art and another rinse after the deoxidizing process, after which a composition in accordance 25 with the present invention may then be coated onto the aluminum in accordance with one of the processes disclosed herein.

The practice of this invention may be further appreciated by consideration of the following, non-limiting, working examples, and the benefits of the invention may be further appreciated by reference to the comparison examples.

## GROUP I

WORKING COMPOSITIONS AND PROCESSES  
USING NECESSARY COMPONENTS (A) AND  
(B), WITH DRY IN PLACE TREATMENTS

## Test Methods and Other General Conditions

Test pieces of Type 3105 aluminum were spray cleaned for 15 seconds at 54.4° C. with an aqueous cleaner containing 45 28 g/L of PARCO® Cleaner 305 (commercially available from the Parker+Amchem Division of Henkel Corp., Madison Heights, Mich., USA). After cleaning, the panels were rinsed with hot water, squeegeed, and dried before roll coating with an acidic aqueous composition as described for 50 the individual examples and comparison examples below.

For this first group of examples and comparison examples, the applied liquid composition according to the invention was flash dried in an infrared oven that produces approximately 49° C. peak metal temperature. Samples thus 55 treated were subsequently coated, according to the recommendations of the suppliers, with various commercial paints as specified further below.

T-Bend tests were according to American Society for Testing materials (hereinafter "ASTM") Method D4145-83; 60 Impact tests were according to ASTM Method D2794-84E1; Salt Spray tests were according to ASTM Method B-117-90 Standard; Acetic Acid Salt Spray tests were according to ASTM Method B-287-74 Standard; and Humidity tests were according to ASTM D2247-8 Standard. The Boiling water immersion test was performed as follows: A 2T bend and a reverse impact deformation were performed on the treated and painted panel. The panel was then immersed for 10

## 13

minutes in boiling water at normal atmospheric pressure, and areas of the panel most affected by the T-bend and reverse impact deformations were examined to determine the percent of the paint film originally on these areas that had not been exfoliated. The rating is reported as a number that is one tenth of the percentage of paint not exfoliated. Thus, the best possible rating is 10, indicating no exfoliation; a rating of 5 indicates 50% exfoliation; etc.

## Specific Compositions

10

## EXAMPLE 1

**5.6** parts of amorphous fumed silicon dioxide  
**396.2** parts of deionized water  
**56.6** parts of aqueous 60% fluotitanic acid (i.e.,  $H_2TiF_6$ )  
**325.4** parts of deionized water  
**216.2** parts of an aqueous solution containing a mixture of  
 4.1 g/l polyacrylic acid and 4.0 g/l polyvinyl alcohol

15 20

## EXAMPLE 2

**58.8** parts of aqueous 60% fluotitanic acid  
**646.0** parts of deionized water  
**5.9** parts of amorphous fumed silicon dioxide  
**10.5** parts of zirconium hydroxide  
**278.8** parts of the 10% solution of water soluble polymer  
 as used in Example 1.

25 30

## EXAMPLE 3

**62.9** parts of aqueous 60% fluotitanic acid  
**330.5** parts of deionized water  
**6.2** parts of amorphous fumed silicon dioxide  
**358.9** parts of deionized water  
**241.5** parts of the 10% water soluble polymer solution as  
 used in Example 1

35 40

## EXAMPLE 4

**56.4** parts of aqueous 60% fluotitanic acid  
**56.4** parts of deionized water  
**2.1** parts of Aerosil™ R-972 (a surface treated dispersed  
 silica)  
**667.0** parts of deionized water  
**218.1** parts of the 10% water soluble polymer solution as  
 used in Example 1

45 50

## EXAMPLE 5

**58.8** parts of aqueous 60% fluotitanic acid  
**3.7** parts of amorphous fumed silicon dioxide  
**10.3** parts of zirconium basic carbonate  
**647.7** parts of deionized water  
**279.5** parts of the 10% solution of water soluble polymer  
 as used in Example 1

55 60 65

## EXAMPLE 6

**52.0** parts of aqueous 60% fluotitanic acid  
**297.2** parts of deionized water  
**3.3** parts of amorphous fumed silicon dioxide  
**9.1** parts of zirconium basic carbonate  
**273.6** parts of deionized water  
**364.8** parts of the 10% solution of water soluble polymer  
 as used in Example 1

## 14

## EXAMPLE 7

**11.0** parts of fumed amorphous silicon dioxide  
**241.0** parts of deionized water  
**114.2** parts of 60% aqueous fluotitanic acid  
**633.8** parts of an aqueous composition prepared from the  
 following ingredients:  
**5.41%** of  $CrO_3$   
**0.59%** of pearlized corn starch  
**94%** of water

## EXAMPLE 8

**666.0** parts of deionized water  
**83.9** parts of 60% aqueous fluotitanic acid  
**5.3** parts of Cab-O-Sil™ M-5 fumed amorphous silicon  
 dioxide  
**14.8** parts of zirconium basic carbonate  
**230.0** parts of RDX 68654™ (also known as RIX  
 95928™) epoxy resin dispersion commercially avail-  
 able from Rhône-Poulenc, containing 40% solids of  
 polymers of predominantly diglycidyl ethers of  
 bisphenol-A, in which some of the epoxide groups have  
 been converted to hydroxy groups and the polymer  
 molecules are phosphate capped

## EXAMPLE 9

**656.0** parts of deionized water  
**183.9** parts of 60% aqueous fluotitanic acid  
**5.3** parts of Cab-O-Sil™ M-5 fumed amorphous silicon  
 dioxide  
**14.8** parts of zirconium basic carbonate  
**240.0** parts of Accumér™ 1510, a commercially available  
 product from Rohm & Haas containing 25% solids of  
 polymers of acrylic acid with a molecular weight of  
 60,000

## EXAMPLE 10

**636.2** parts of deionized water  
**83.7** parts of 60% aqueous fluotitanic acid  
**5.3** parts of Cab-O-Sil™ M-5 fumed amorphous silicon dioxide  
**14.6** parts of zirconium basic carbonate  
**37.6** parts of the 10% solution of water soluble polymer  
 as used in Example 1  
**222.6** parts of Accumér™ 1510, a commercially available  
 product from Rohm & Haas containing 25% solids of  
 polymers of acrylic acid with a molecular weight of  
 60,000

For each of Examples 1–6 and 8–10, the ingredients were added in the order indicated to a container provided with stirring. (Glass containers are susceptible to chemical attack by the compositions and generally should not be used, even on a laboratory scale; containers of austenitic stainless steels such as Type 316 and containers made of or fully lined with resistant plastics such as polymers of tetrafluoroethylene or chlorotrifluoroethylene have proved to be satisfactory.) In each of these Examples except Example 4, after the addition of the silica component and before the addition of the subsequently listed components, the mixture was heated to a temperature in the range from 38°–43° C. and maintained within that range of temperatures for a time of 20–30 minutes. Then the mixture was cooled to a temperature below 30° C., and the remaining ingredients were stirred in without additional heating, until a clear solution was obtained after each addition.

For Example 4, the  $\text{SiO}_2$  used was surface modified with a silane, and because of its hydrophobic nature, the mixture containing this form of silica was heated for 1.5 hours at 70° C. to achieve transparency. The remaining steps of the process were the same as for Example 1.

For Example 7, the first three ingredients listed were mixed together and maintained at 40°±5° C. for 20–30 minutes with stirring and then cooled. In a separate container, the  $\text{CrO}_3$  was dissolved in about fifteen times its own weight of water, and to this solution was added a slurry of the corn starch in twenty-four times its own weight of water. The mixture was then maintained for 90 minutes with gentle stirring at 88°±6° C. to reduce part of the hexavalent chromium content to trivalent chromium. Finally, this mixture was cooled with stirring and then added to the previously prepared heated mixture of fluotitanic acid, silicon dioxide, and water. This composition is used in the manner known in the art for compositions containing hexavalent and trivalent chromium and dispersed silica, but it is much more stable to storage without phase separation.

#### Comparative Example 1

18.9 parts of aqueous 60% fluotitanic acid  
363.6 parts of the 10% solution of water soluble polymer as used in Example 1  
617.5 parts of deionized water

#### Comparative Example 2

18.9 parts of aqueous 60% fluotitanic acid  
71.8 parts of the 10% solution of water soluble polymer as used in Example 1  
909.3 parts of deionized water

For Comparative Examples 1 and 2 the components were added together with agitation in the order indicated, with no heating before use in treating metal surfaces.

Add-on mass levels, specific paints used, and test results with some of the compositions described above are shown in Tables 1–5 below.

TABLE 1

| Panels Painted with PPG Duracron™ 1000 White Single Coat Acrylic Paint |               |        |                                                     |                           |           |                    |
|------------------------------------------------------------------------|---------------|--------|-----------------------------------------------------|---------------------------|-----------|--------------------|
| Treatment                                                              | Boiling Water |        | Coating Weight                                      | HAc Salt Spray            | 504 Hours | Humidity 1008 Hrs. |
|                                                                        | 2T Bend       | Impact |                                                     |                           |           |                    |
| Example 1                                                              | 9             | 10     | 65 mg/m <sup>2</sup><br>as Ti<br>s 0–1 <sup>s</sup> | e 0–1 <sup>s</sup><br>Vf9 |           |                    |
| "                                                                      | 9             | 10     | 43 mg/m <sup>2</sup><br>as Ti<br>s 0–1 <sup>s</sup> | e 0–1 <sup>s</sup><br>Vf9 |           |                    |
| Comparative Example 1                                                  | 5             | 7      | 39 mg/m <sup>2</sup><br>as Ti<br>s 0–2 <sup>s</sup> | D9                        |           |                    |
| Comparative Example 1                                                  | 0             | 0      | 27 mg/m <sup>2</sup><br>as Ti<br>s 0–2 <sup>s</sup> | D9                        |           |                    |
| Comparative Example 2                                                  | 7             | 8      | 65 mg/m <sup>2</sup><br>as Ti<br>s 0–1 <sup>s</sup> | Vf9                       |           |                    |
| Comparative Example 2                                                  | 4             | 6      | 29 mg/m <sup>2</sup><br>as Ti<br>s 0–1 <sup>s</sup> | Fm9                       |           |                    |

TABLE 2

| Panels Painted with Lilly™ Black Single Coat Polyester |               |        |                                                     |                           |                           |                    |
|--------------------------------------------------------|---------------|--------|-----------------------------------------------------|---------------------------|---------------------------|--------------------|
| Treatment                                              | Boiling Water |        | Coatin                                              | HAc Salt Spray 504 Hours  | Salt Spray 1008 Hours     | Humidity 1008 Hrs. |
|                                                        | 2T Bend       | Impact |                                                     |                           |                           |                    |
| Example 2                                              | 10            | 10     | 54 mg/m <sup>2</sup><br>as Ti<br>s 0–1 <sup>s</sup> | e 0–1 <sup>s</sup><br>s N | e N                       | Vf9                |
| Example 3                                              | 10            | 10     | 64 mg/m <sup>2</sup><br>as Ti<br>s 0–2 <sup>s</sup> | e 0–2 <sup>s</sup><br>s N | e 0–1 <sup>s</sup><br>e N | Vf9                |

TABLE 3

| Panels Painted with Lilly™ Colonial White Single Coat Polyester |               |        |                                      |                                          |                           |                    |
|-----------------------------------------------------------------|---------------|--------|--------------------------------------|------------------------------------------|---------------------------|--------------------|
| Treatment                                                       | Boiling Water |        | Coating Weight                       | HAc Salt Spray 504 Hours                 | Salt Spray 1008 Hours     | Humidity 1008 Hrs. |
|                                                                 | 2T Bend       | Impact |                                      |                                          |                           |                    |
| Example 4                                                       | 5             | 8      | 65 mg/m <sup>2</sup><br>as Ti<br>s N | e N<br>s N                               | e N                       | Vf9                |
| Example 5                                                       | 10            | 10     | 22 mg/m <sup>2</sup><br>as Ti<br>s N | e N<br>s N                               | e N<br>s N                | Vf9                |
| Example 5                                                       | 10            | 10     | 54 mg/m <sup>2</sup><br>as Ti<br>s N | e N<br>s N                               | e N<br>s N                | Vf9                |
| Example 6                                                       | 10            | 10     | 22 mg/m <sup>2</sup><br>as Ti<br>s N | e 0–1 <sup>s</sup><br>s N                | e N<br>s N                | Vf9                |
| Example 6                                                       | 10            | 10     | 54 mg/m <sup>2</sup><br>as Ti<br>s N | e 0–1 <sup>s</sup><br>s N                | e N<br>s N                | Vf9                |
| Example 8                                                       | 9.8           | 10     | 12 mg/m <sup>2</sup><br>as Ti<br>s N | e N<br>s 0–1 <sup>s</sup>                | e N<br>s N                | N                  |
| Example 8                                                       | 9.6           | 10     | 24 mg/m <sup>2</sup><br>as Ti<br>s N | e N<br>s 0–1 <sup>s</sup>                | e N<br>s N                | N                  |
| Example 9                                                       | 10            | 10     | 11 mg/m <sup>2</sup><br>as Ti<br>s N | e N<br>s 0–1 <sup>s</sup>                | e N<br>s 0–1 <sup>s</sup> | N                  |
| Example 9                                                       | 9.8           | 10     | 24 mg/m <sup>2</sup><br>as Ti<br>s N | e 0–1 <sup>s</sup><br>s 0–1 <sup>s</sup> | e N<br>s 0–1              | N                  |
| Example 10                                                      | 9.8           | 9.8    | 17 mg/m <sup>2</sup><br>as Ti<br>s N | e 0–1 <sup>s</sup><br>s 0–1 <sup>s</sup> | e N<br>s N                | Vf9                |
| Example 10                                                      | 9.9           | 10     | 25 mg/m <sup>2</sup><br>as Ti<br>s N | e 0–1 <sup>s</sup><br>s 0–1 <sup>s</sup> | e N<br>s N                | Vf9                |
| Example 10                                                      | 9.9           | 10     | 33 mg/m <sup>2</sup><br>as Ti<br>s N | e 0–1 <sup>s</sup><br>s 0–1 <sup>s</sup> | e N<br>s N                | Vf9                |

TABLE 4

| Panels Painted with Valspar/Desoto™ White Single Coat Polyester |               |        |                                                     |                           |                           |                    |
|-----------------------------------------------------------------|---------------|--------|-----------------------------------------------------|---------------------------|---------------------------|--------------------|
| Treatment                                                       | Boiling Water |        | Coating Weight                                      | HAc Salt Spray 504 Hours  | Salt Spray 1008 Hours     | Humidity 1008 Hrs. |
|                                                                 | 2T Bend       | Impact |                                                     |                           |                           |                    |
| Example 2                                                       | 10            | 10     | 39 mg/m <sup>2</sup><br>as Ti<br>s 0–1 <sup>s</sup> | e 0–1 <sup>s</sup><br>s N | e N                       | Vf9                |
| Example 2                                                       | 10            | 10     | 48 mg/m <sup>2</sup><br>as Ti<br>s 0–1 <sup>s</sup> | e 0–1 <sup>s</sup><br>e N | e N                       | Vf9                |
| Example 2                                                       | 10            | 10     | 70 mg/m <sup>2</sup><br>as Ti<br>s 0–1 <sup>s</sup> | e 0–2 <sup>s</sup><br>s N | e N                       | Vf9                |
| Example 2                                                       | 10            | 10     | 87 mg/m <sup>2</sup><br>as Ti<br>s 0–1 <sup>s</sup> | e N<br>s N                | e 0–1 <sup>s</sup><br>e N | Vf9                |
| Example 3                                                       | 10            | 10     | 29 mg/m <sup>2</sup><br>as Ti<br>s 0–1 <sup>s</sup> | e 0–2 <sup>s</sup><br>s N | e N                       | Vf9                |
| Example 3                                                       | 10            | 10     | 42 mg/m <sup>2</sup><br>as Ti<br>s 0–1 <sup>s</sup> | e 0–1 <sup>s</sup><br>s N | e N                       | Vf9                |
| Example 3                                                       | 10            | 10     | 57 mg/m <sup>2</sup><br>as Ti<br>s 0–1 <sup>s</sup> | e 0–1<br>s N              | e N                       | Vf9                |
| Example 3                                                       | 10            | 10     | 82 mg/m <sup>2</sup><br>as Ti<br>s 0–2 <sup>s</sup> | e 0–2 <sup>s</sup><br>s N | e 0–1 <sup>s</sup><br>Vf9 | Vf9                |

TABLE 4-continued

| Panels Painted with Valspar/Desoto™ White Single Coat Polyester |               |        |                               |                                          |            |                    |
|-----------------------------------------------------------------|---------------|--------|-------------------------------|------------------------------------------|------------|--------------------|
| Treatment                                                       | Boiling Water |        | HAc Salt                      |                                          | Salt Spray |                    |
|                                                                 | 2T Bend       | Impact | Coating Weight                | Spray 504 Hours                          | 1008 Hours | Humidity 1008 Hrs. |
| Example 4                                                       | 7             | 10     | 65 mg/m <sup>2</sup><br>as Ti | e 0-1 <sup>s</sup><br>s 0-1 <sup>s</sup> | e N<br>s N | Vf <sup>9</sup>    |

TABLE 5

| Panels Painted with Valspar™ Colonial White Single Coat Polyester |               |        |                               |                           |                                          |                    |
|-------------------------------------------------------------------|---------------|--------|-------------------------------|---------------------------|------------------------------------------|--------------------|
| Treatment                                                         | Boiling Water |        | HAc Salt                      |                           | Salt Spray                               |                    |
|                                                                   | 2T Bend       | Impact | Coating Weight                | Spray 504 Hours           | 1008 Hours                               | Humidity 1008 Hrs. |
| Example 2                                                         | 10            | 10     | 54 mg/m <sup>2</sup><br>as Ti | e N<br>s N                | e N<br>s N                               | Fm <sup>9</sup>    |
| Example 3                                                         | 10            | 10     | 64 mg/m <sup>2</sup><br>as Ti | e 0-1 <sup>s</sup><br>s N | e 0-1 <sup>s</sup><br>s 0-1 <sup>s</sup> | Fm <sup>9</sup>    |

The storage stability of the compositions according to all of the examples above except Example 2 was so good that no phase separation could be observed after at least 1500 hours of storage. For Example 2, some settling of a slight amount of apparent solid phase was observable after 150 hours.

## GROUP II

### TREATMENT WITH COMPOSITIONS CONTAINING NECESSARY COMPONENTS (A) AND (B), WITH SUBSEQUENT RINSING

To obtain the results reported below, an alternative process of treating the metal surfaces according to the invention and different aluminum alloys were used. Specifically, in part I of this Group, test pieces of Type 5352 or 5182 aluminum were spray cleaned for 10 seconds at 54.4° C. with an aqueous cleaner containing 24 g/L of PARCO® Cleaner 305 (commercially available from the Parker+Amchem Division of Henkel Corp., Madison Heights, Mich., USA). After cleaning, the panels were rinsed with hot water; then they were sprayed with the respective treatment solutions according to the invention, which were the same as those already described above with the same Example Number, except that they were further diluted with water to the concentration shown in the tables below, for 5 seconds; and then were rinsed successively with cold tap water and deionized water and dried, prior to painting.

The “0T Bend” column in the following tables reports the result of a test procedure as follows:

1. Perform a 0-T bend in accordance with ASTM Method D4145-83.
2. Firmly apply one piece of #610 Scotch® tape to the area of the test panel with the 0-T bend and to the adjacent flat area.
3. Slowly pull the tape off from the bend and the adjacent flat area.
4. Repeat steps 2 and 3, using a fresh piece of tape for each repetition, until no additional paint is removed by the tape.

5. Report the maximum distance from the 0-T bend into the flat area from which paint removal is observed according to the scale below:

| 5  | Paint loss in mm | Rating |
|----|------------------|--------|
| 10 | 0                | 5.0    |
|    | 0.20             | 4.9    |
|    | 0.30             | 4.8    |
|    | 0.8              | 4.5    |
|    | 1.6              | 4.0    |
|    | 2.4              | 3.5    |
|    | 3.2              | 3.0    |
|    | 4.0              | 2.5    |
|    | 4.8              | 2.0    |
|    | 5.6              | 1.5    |
| 15 | 6.4              | 1.0    |
|    | 7.2              | 0.5    |
|    | >7.2             | 0      |

The “Ninety Minute Steam Exposure” columns of the tables below report the results of tests performed as follows:

1. Expose the painted samples to steam at a temperature of 120° C. steam for 90 minutes in a pressure cooker or autoclave.
2. Crosshatch the painted sample—two perpendicular cuts; a Gardner crosshatch tool with 11 knife edges spaced 1.5 mm apart was used.
3. Firmly apply #610 Scotch™ tape to the crosshatched area and remove tape.
4. Examine the crosshatched area for paint not removed by the tape and report a number representing one-tenth of the percentage of paint remaining.
5. Using a microscope at 10-80 times magnification, visually observe crosshatched area for blistering, and rate size and density of blisters.

The “15 Minute Boiling DOWFAX™ 2A1 Immersion” columns of the tables below report the results of tests performed after treatment as follows:

1. Prepare solution of 1% by volume of DOWFAX™ 2A1 in deionized water and bring to boil.
2. Immerse painted test panels in the boiling solution prepared in step 1 and keep there for 15 minutes; then remove panels, rinse with water, and dry.

DOWFAX™ 2A1 is commercially available from Dow Chemical and is described by the supplier as 45% active sodium dodecyl diphenyloxide disulfonate. The “Cross Hatch” test after this treatment was made in the same way as described above for steps 2-4 after “Ninety Minute Steam Exposure”. The “Reverse Impact” test was made as described in ASTM D2794-84E1 (for 20 inch pounds impact), then proceeding in the same way as described above for steps 3-4 after “Ninety Minute Steam Exposure”.

5. The “Feathering” test was performed as follows: Using a utility knife, scribe a slightly curved “V” on the back side of the test panel. Using scissors, cut up about 12 millimeters from the bottom along the scribe. Bend the inside of the V away from side for testing. Place sample in a vise and, using pliers, pull from the folded section with a slow continuous motion. Ignore the part of the panel between the top edges nearest to the vertex and a line parallel to the top edge but 19 mm away from it. On the remainder of the panel, measure to edge of feathering in millimeters. Record the largest value observed.

The results of tests according to these procedures are shown in Tables 6-8 below.

TABLE 6

5352 Alloy Panels Painted with Valspar™ S-9009-139 Paint

| Invention                               | Composition | Concen-<br>tration | pH                                 | Coating<br>Weight | Ninety Minute<br>Steam Exposure |                |                                  |
|-----------------------------------------|-------------|--------------------|------------------------------------|-------------------|---------------------------------|----------------|----------------------------------|
|                                         |             |                    |                                    |                   | OT Bend                         | Cross<br>Hatch | Blis-<br>tering                  |
| Example 1                               | 1%          | 2.7                | 4.0<br>mg/m <sup>2</sup><br>as Ti  |                   | 5                               | 10             | Very<br>few,<br>small-<br>medium |
| Example 1                               | 1%          | 3.2                | 11.4<br>mg/m <sup>2</sup><br>as Ti |                   | 5                               | 10             | few,<br>small                    |
| Example 1                               | 3%          | 2.5                | 2.3<br>mg/m <sup>2</sup><br>as Ti  |                   | 5                               | 10             | very<br>few,<br>very<br>small    |
| Clean<br>only<br>(Com-<br>pari-<br>son) | N/A         |                    |                                    |                   | 1.5                             | 10             | few,<br>medium                   |

TABLE 7

5352 Alloy Panels Painted with Valspar™ S-9009-154 Paint

| Invention | Composition | Concen-<br>tration | pH                                | Coating<br>Weight | Ninety Minute<br>Steam Exposure |                |                               |
|-----------|-------------|--------------------|-----------------------------------|-------------------|---------------------------------|----------------|-------------------------------|
|           |             |                    |                                   |                   | OT Bend                         | Cross<br>Hatch | Blis-<br>tering               |
| Example 1 | 1%          | 2.9                | 4.2<br>mg/m <sup>2</sup><br>as Ti |                   | 5                               | 9-10           | Very<br>few,<br>small         |
| Example 1 | 3%          | 2.7                | 2.6<br>mg/m <sup>2</sup><br>as Ti |                   | 5                               | 9-10           | very<br>few,<br>very<br>small |

TABLE 8

5182 alloy panels Painted with Valspar™ S-9835002 Paint

| Invention | Composition     | Concen-<br>tration | pH                                | Coating<br>Weight | 15 Minute Boiling<br>DOWFAX™ 2A1 Immersion |                   |            |
|-----------|-----------------|--------------------|-----------------------------------|-------------------|--------------------------------------------|-------------------|------------|
|           |                 |                    |                                   |                   | Cross<br>Hatch                             | Reverse<br>Impact | Feathering |
| Example 1 | 1% by<br>weight | 2.9                | 7.9<br>mg/m <sup>2</sup><br>as Ti |                   | 10                                         | 10                | 0.35 mm    |

In part II of this Group, Type 5352 aluminum was used, and the process sequence used in part I, except for final drying, was used but was then followed by passing the test pieces, still wet from the deionized water rinse after contact with a composition according to this invention, through power driven squeegee rolls arranged so that the test pieces passed through the squeegee rolls in a horizontal position immediately after being sprayed liberally with the final treatment liquid composition at a temperature of 60° C. before being dried. In Examples 11 and 13 the treatment liquid in this final stage was simply deionized water with a conductivity of not more than 4.0  $\mu$ Siemens/cm, while in Example 12 the treatment liquid in this final stage was obtained by mixing 35 ml of Parcolene™ 95AT and 2.0 ml of Parcolene™ 88B with 7 liters of deionized water and had a pH of 5.18 and a conductivity of 56  $\mu$ Siemens/cm. (Both

Parcolene™ products noted are commercially available from the Parker+Amchem Div. of Henkel Corp., Madison Heights, Mich.) This latter type of final treatment liquid is an example of one containing polymers and/or copolymers of one or more x-(N—R<sup>1</sup>—N—R<sup>2</sup>-aminomethyl)-4-hydroxy-styrenes as already described above.

Concentrate II-II used in each of Examples 11-13 had the following composition:

1892.7 parts of deionized water  
10 83.7 parts of 60% aqueous fluotitanic acid  
5.3 parts of Cab-O-Sil™ M-5 fumed amorphous silicon dioxide  
18.3 parts of zirconium basic carbonate.

These ingredients were simply mixed together with mechanical agitation in the order shown, with a pause after each addition until the solution became optically clear. Although the partial mixture was not transparent immediately after addition of the silicon dioxide, it became clear after a few minutes of mixing, even without any heating.

20 The working solution for Examples 11 and 12 was prepared by diluting 200 grams of the concentrate II-II, along with sufficient sodium carbonate to result in a pH of 2.92±0.2, to form 6 liters of working composition. For Example 13, the working solution was made in the same 25 way, except that it also contained 5 grams of a concentrated polymer solution made according to the directions of column 11 lines 39-49 of U.S. Pat. No. 4,963,596, except as follows: The preparation was carried out on a substantially larger scale; the proportions of ingredients were changed to the following: 241 parts of Propasol™ P, 109 parts of Resin M, 179 parts of N-methylglucamine, 73.5 parts of aqueous 37% formaldehyde, and 398 parts of deionized water, of which 126 parts were reserved for a final addition not described in the noted patent, with the remainder used to slurry the N-methylglucamine as noted in the patent; and the temperature noted as 60°-65° C. in the patent was reduced to 57° C.

25 The dried test panels were then coated with Valspar™ 9009-157 paint according to the directions of the paint 30 supplier, and the paint coated panels were tested as described for the tests of the same name in part I of Group II. Results are shown in Table 9.

TABLE 9

| Example | 90 Minute Steam Exposure |                         |          |             |
|---------|--------------------------|-------------------------|----------|-------------|
|         | Number                   | mg of Ti/m <sup>2</sup> | O-T Bend | Cross Hatch |
| 11      | 3.6                      | 4.5                     | 10       | 4.5         |
| 12      | 4.6                      | 4.9                     | 10       | 4.5         |
| 13      | 5.4                      | 4.8                     | 10       | 4.0         |

45 In part III of Group II, Type 2024-T3 aluminum alloy was used as the substrate metal to be treated according to the 55 invention. Test panels of this alloy were cleaned by immersion for 3 minutes at 65° C. in an aqueous solution containing 15 grams per liter (hereinafter usually abbreviated as "g/L") of RIDOLENE® 53 Cleaner concentrate, a commercial silicated alkaline cleaner product available from the Parker Amchem Division of Henkel Corp., Madison Heights, Mich. USA, then rinsed in hot water, then deoxidized by immersion for 5 minutes in a liquid composition of Deoxidizer 6-16, commercially available from the Parker Amchem Division of Henkel Corp., Madison Heights, Mich. 60 USA, then rinsed in cold water, then immersed at 27° C. in a working composition according to the invention that had been prepared as follows: 24.1 grams of aqueous fluotitanic 65

## 21

acid containing 60% of  $H_2TiF_6$ , 9.5 grams of solid zirconium basic carbonate containing 40% of Zr, 3.4 grams of amorphous silicon dioxide (Cab-O-Sil™ M-5, commercially available from Cabot Corp., and 168.5 grams of deionized water were agitated together at a temperature of 40° C. for a time of 30 minutes, so that a liquid composition with no visible settling of solids therefrom was produced. This liquid composition was then diluted with 2 liters of deionized water, and 0.12 grams of sodium chloride, 5.83 grams of sodium nitrate, and 27.6 grams of sodium dichromate dihydrate were then dissolved in this diluted mixture. Finally, the volume of the mixture was increased to 3.9 liters by adding more deionized water.

Panels that had been cleaned, rinsed, deoxidized, and again rinsed as described above were immersed in the composition noted in the immediately preceding paragraph while this composition was maintained at 27° C. for either 3 or 5 minutes. Resulting coating mass add-ons were 130 and 140 mg/m<sup>2</sup> respectively. After exposure to 436 hours of salt spray testing according to American Society for Testing and Materials Test, panels exposed for both intervals of time had no visible pits or discoloration.

GROUP III, WITH NECESSARY COMPONENTS  
(A) AND (B')

## EXAMPLE 14

A first concentrate was made by mixing 750 parts of tap water and 274 parts of Acrysol™ A-1, a commercially available product from Rohm and Haas containing 25% solids of polymers of acrylic acid with a molecular weight of less than 50,000. A second concentrate was made by mixing, in a container separate from that used for the first concentrate 951.3 parts of tap water and 66.7 g/l of Gohsenol™ GLO-5, a commercially available product from Nippon Gohsei which is a low molecular weight polyvinyl alcohol; the latter was added to the tap water with stirring at a slow and controlled flow, after which the temperature was increased to 49°–54° C. for 30 minutes with slow stirring until all was dissolved.

An amount of these concentrates equal, for each concentrate separately, to 6 volume % of the final volume of composition ready for treating a metal surface according to this invention, was then added with stirring at ambient temperature to a large excess of water, and after addition of both concentrates, additional water was added to reach the final volume of treatment composition, which contained 4.1 g/l of polyacrylic acid and 4.0 g/l of polyvinyl alcohol.

This composition was then contacted with an aluminum surface by dipping or spraying for a time from 30 to 60 seconds, after which time the surfaces treated were removed from contact with the treating composition, allowed to dry in the ambient atmosphere without rinsing, and then baked in a warm air oven at 88° C. for 5 minutes to simulate commercial operating conditions. The surfaces thus prepared were painted with conventional paints.

## EXAMPLES 15–20

In each of these examples, the treating composition is prepared in the same general manner as in Example 14, by making separate concentrates of the hydroxyl group containing polymer and polyacrylic acid components, mixing an appropriate amount of these concentrates with a larger volume of water, adding any additional components used, and finally adjusting to the final desired volume or mass by the addition of more water. These compositions are then

## 22

applied to aluminum surfaces in the same manner as described for Example 14. The specific active ingredients and concentrations or amounts thereof in the treatment composition for each example are as follows:

## EXAMPLE 15

4.1 g/l of Acrysol™ A-1; 4.0 g/l of Gohsenol™ GLO-5; and 1.2 g/l of hexafluorozirconic acid.

## EXAMPLE 16

4.1 g/l of Acrysol™ A-1 and 0.6 g/l of polyethylene glycol having a molecular weight of less than about 600,000.

## EXAMPLE 17

4.1 g/l of Acrysol™ A-1; 0.6 g/l of polyethylene glycol having a molecular weight of less than about 600,000; and 1.2 g/l of hexafluorozirconic acid.

## EXAMPLE 18

4.1 g/l of Acrysol™ A-1 and 0.8 g/l of dextrin.

## EXAMPLE 19

4.1 g/l of Acrysol™ A-1; 0.8 g/l of dextrin; and 1.2 g/l of hexafluorotitanic acid.

## EXAMPLE 20

651.4 parts of deionized water; 83.7 parts of 60% aqueous fluotitanic acid; 5.3 parts of Cab-O-Sil™ M-5 fumed amorphous silicon dioxide; 14.6 parts of zirconium basic carbonate; 200.0 parts of Accumer™ 1510, a commercially available product from Rohm and Haas containing 25% solids of polymers of acrylic acid with a molecular weight of about 60,000; and 55.0 parts of Gohsenol™ GLO-5.

The invention claimed is:

1. A process for making a liquid metal treating composition, said process comprising steps of:

(I) providing a precursor mixture with a continuous liquid phase, said precursor mixture consisting essentially of water and:

(A) a dissolved component selected from the group consisting of  $H_2TiF_6$ ,  $H_2ZrF_6$ ,  $H_2HF_6$ ,  $H_2SiF_6$ ,  $H_2GeF_6$ ,  $H_2SnF_6$ ,  $HBF_4$ , and mixtures thereof and

(B) a dissolved, dispersed, or both dissolved and dispersed component selected from the group consisting of Ti, Zr, Hf, Al, Si, Ge, Sn, and B, the oxides, hydroxides, and carbonates of Ti, Zr, Hf, Al, Si, Ge, Sn, and B, and mixtures of any two or more of these elements, oxides, hydroxides, and carbonates,

said precursor mixture having at least one of the following characteristics: (i) it is not optically transparent in a thickness of 1 cm; (ii) it scatters visible light; or (iii) it undergoes visually detectable settling of a solid phase if maintained for at least 100 hours at a temperature between its freezing point and 20° C.;

(II) maintaining the precursor liquid mixture provided in step (I) for at least a sufficient time at a sufficient temperature to form a stabilized liquid mixture that is free from any visually observable evidence of phase separation, is transparent when viewed in a thickness of 1 cm, and is sufficiently stable that it would remain free from any visually observable evidence of phase separation during storage at any temperature in the range from 20° to 25° C. for a period of at least 100 hours; and

## 23

- (III) mixing with the stabilized liquid mixture from the end of step (II):
- (C) a component selected from the group consisting of water soluble compounds containing hexavalent chromium; and, optionally, one or more of water and;
- (D) a component selected from the group consisting of water soluble oxides, carbonates, and hydroxides of all of the elements Ti, Zr, Hf, B, Al, Si, Ge, and Sn; and
- (E) a component selected from the group consisting of water soluble oxidizing agents that are not part of any of the previously recited components,

to form said liquid metal treating composition, which is sufficiently stable that it remains free from any visually observable evidence of phase separation during storage at temperature in the range from 20+ to 25° C. for a period of at least 100 hours and which contains; (i) a total concentration of titanium, zirconium, hafnium, boron, aluminum, silicon, germanium, and tin derived from component (A) of the precursor mixture that is from about 1.0 to about 200 mM/L and (ii) an amount of hexavalent chromium that has a molar ratio to all metalloid and metal atoms derived from components (A) and (B) that is in a range from about 0.3:1.0 to about 10:1.0.

2. A liquid metal treating composition made by a process according to claim 1.

3. A process for forming a corrosion protective coating layer on a metal surface, said process comprising steps of:

- (IV) contacting the metal surface with a liquid metal treating composition according to claim 2 at a temperature in the range from about 15° to about 90° C. for a time in the range from about 1 to about 1800 seconds;
- (V) removing the metal surface from contact with said liquid metal treatment composition;
- (VI) rinsing said metal surface with water; and, optionally, one or both of:
- (VII) rinsing the metal surface after step (VI) with an aqueous composition comprising polymers of one or more  $x\text{-(N-}R^1\text{-N-}R^2\text{-aminomethyl)-4-hydroxy-}$  styrenes, where  $x=2, 4, 5$ , or  $6$ ,  $R^1$  represents an alkyl group containing from 1 to 4 carbon atoms and  $R^2$  represents a substituent group conforming to the general formula  $\text{H}(\text{CHOH})_n\text{CH}_2-$ , where  $n$  is an integer from 1 to 7; and

(VIII) drying the rinsed metal surface.

4. A process according to claim 1, wherein: (i) the precursor mixture contains from about 0.08 to about 3 M/kg of component (A) and (ii) component (B) in the precursor mixture includes silicon and zirconium in amounts such that there is a ratio of total moles of component (A) to total moles of component (B) in the range from 0.05:1.0 to 5.0:1.0 and there is a ratio of moles of silicon to moles of zirconium in the range from 0.5:1.0 to 5:1.0.

5. A process for forming a corrosion protective coating layer on a metal surface, said process comprising steps of:

- (IV) contacting the metal surface with a liquid metal treating composition according to claim 1 at a temperature in the range from about 18° to about 60° C. for a time in the range from about 30 to about 1200 seconds;
- (V) removing the metal surface from contact with said liquid metal treatment composition;
- (VI) rinsing said metal surface with water; and, optionally, one or both of:
- (VII) rinsing the metal surface after step (VI) with an aqueous composition comprising polymers of one or

## 24

more  $x\text{-(N-}R^1\text{-N-}R^2\text{-aminomethyl)-4-hydroxy-}$  styrenes, where  $x=2, 4, 5$ , or  $6$ ,  $R^1$  represents an alkyl group containing from 1 to 4 carbon atoms and  $R^2$  represents a substituent group conforming to the general formula  $\text{H}(\text{CHOH})_n\text{CH}_2-$ , where  $n$  is an integer from 1 to 7; and

(VIII) drying the rinsed metal surface.

6. A process according to claim 4, wherein: (i) the precursor mixture contains from about 0.12 to about 2.0 M/kg of  $\text{H}_2\text{TiF}_6$ ; (ii) the ratio of total moles of component (A) to total moles of component (B) is in the range from 0.20:1.0 to 3.0:1.0 and (iii) the ratio of moles of silicon to moles of zirconium is in the range from 0.9:1.0 to 3.0:1.0.

7. A liquid metal treating composition made by a process according to claim 6, wherein titanium derived from component (A) of the precursor mixture is present in a total concentration from about 4.0 to about 100 mM/L and (ii) hexavalent chromium is present in an amount having a molar ratio to titanium, silicon, and zirconium atoms derived from components (A) and (B) in the range from about 0.7:1.0 to about 6:1.0.

8. A process for forming a corrosion protective coating layer on a metal surface, said process comprising steps of:

(IV) contacting the metal surface with a liquid metal treating composition according to claim 7 at a temperature in the range from about 18° to about 40° C. for a time in the range from about 30 to about 600 seconds;

(V) removing the metal surface from contact with said liquid metal treatment composition;

(VI) rinsing said metal surface with water; and, optionally, one or both of:

(VII) rinsing the metal surface after step (VI) with an aqueous composition comprising polymers of one or more  $x\text{-(N-}R^1\text{-N-}R^2\text{-aminomethyl)-4-hydroxy-}$  styrenes, where  $x=2, 4, 5$ , or  $6$ ,  $R^1$  represents an alkyl group containing from 1 to 4 carbon atoms and  $R^2$  represents a substituent group conforming to the general formula  $\text{H}(\text{CHOH})_n\text{CH}_2-$ , where  $n$  is an integer from 1 to 7; and

(VIII) drying the rinsed metal surface.

9. A process according to claim 6, wherein: (i) the precursor mixture contains from about 0.27 to about 1.0 M/kg of  $\text{H}_2\text{TiF}_6$ ; (ii) the ratio of total moles of component (A) to total moles of component (B) is in the range from 0.40:1.0 to 2.0:1.0; and (iii) the ratio of moles of silicon to moles of zirconium is in the range from 1.1:1.0 to 2.7:1.0.

10. A liquid metal treating composition made by a process according to claim 9, wherein: (i) titanium derived from component (A) of the precursor mixture is present in a total concentration from about 8.0 to about 60 mM/L; (ii) hexavalent chromium is present in an amount having a molar ratio to titanium, silicon, and zirconium atoms derived from components (A) and (B) in the range from about 0.80:1.0 to about 4.0:1.0; (iii) a concentration of nitrate ions in the range from about 1 to about 100 mM/L is present; and (iv) a concentration of halide ions in the range from about 0.01 to about 50 mM/L is present.

11. A process for forming a corrosion protective coating layer on a metal surface, said process comprising steps of:

(IV) contacting the metal surface with a liquid metal treating composition according to claim 10 at a temperature in the range from about 21° to about 35° C. for a time in the range from about 50 to about 300 seconds;

(V) removing the metal surface from contact with said liquid metal treatment composition;

(VI) rinsing said metal surface with water; and, optionally, one or both of:

## 25

(VII) rinsing the metal surface after step (VI) with an aqueous composition comprising polymers of one or more  $x$ -(N—R<sup>1</sup>—N—R<sup>2</sup>-aminomethyl)-4-hydroxystyrenes, where  $x=2, 4, 5$ , or  $6$ , R<sup>1</sup> represents an alkyl group containing from 1 to 4 carbon atoms and R<sup>2</sup> represents a substituent group conforming to the general formula H(CHOH)<sub>n</sub>CH<sub>2</sub>—, where n is an integer from 1 to 7; and

(VIII) drying the rinsed metal surface.

12. A process according to claim 9, wherein: (i) the precursor mixture contains from about 0.31 to about 0.80 M/kg of H<sub>2</sub>TiF<sub>6</sub>; (ii) the ratio of total moles of component (A) to total moles of component (B) is in the range from 0.60:1.0 to 1.5:1.0; and (iii) the ratio of moles of silicon to moles of zirconium is in the range from 1.1:1.0 to 2.7: 1.0.

13. A liquid metal treating composition made by a process according to claim 12, wherein: (i) titanium derived from component (A) of the precursor mixture is present in a total concentration from about 12 to about 40 mM/L; (ii) hexavalent chromium is present in an amount having a molar ratio to titanium, silicon, and zirconium atoms derived from components (A) and (B) in the range from about 0.90:1.0 to about 2.4: 1.0; (iii) a concentration of nitrate ions in the range from about 4 to about 40 mM/L is present; and (iv) a concentration of halide ions in the range from about 0.01 to about 50 mM/L is present.

14. A process for forming a corrosion protective coating layer on a metal surface, said process comprising steps of:

(IV) contacting the metal surface with a liquid metal treating composition according to claim 13 at a temperature in the range from about 21° to about 32° C. for a time in the range from about 75 to about 300 seconds;

(V) removing the metal surface from contact with said liquid metal treatment composition;

(VI) rinsing said metal surface with water; and, optionally, one or both of:

(VII) rinsing the metal surface after step (VI) with an aqueous composition comprising polymers of one or more  $x$ -(N—R<sup>1</sup>—N—R<sup>2</sup>-aminomethyl)-4-hydroxystyrenes, where  $x=2, 4, 5$ , or  $6$ , R<sup>1</sup> represents an alkyl group containing from 1 to 4 carbon atoms and R<sup>2</sup> represents a substituent group conforming to the general formula H(CHOH)<sub>n</sub>CH<sub>2</sub>—, where n is an integer from 1 to 7; and

(VIII) drying the rinsed metal surface.

15. A process according to claim 12, wherein: (i) the precursor mixture contains from about 0.360 to about 0.60 M/kg of H<sub>2</sub>TiF<sub>6</sub>; (ii) the ratio of total moles of component (A) to total moles of component (B) is in the range from 0.70:1.0 to 1.2:1.0; and (iii) the ratio of moles of silicon to moles of zirconium is in the range from 1.50:1.0 to 2.3:1.0.

## 26

16. A liquid metal treating composition made by a process according to claim 15, wherein: (i) titanium derived from component (A) of the precursor mixture is present in a total concentration from about 16 to about 35 mM/L; (ii) hexavalent chromium is present in an amount having a molar ratio to titanium, silicon, and zirconium atoms derived from components (A) and (B) in the range from about 1.00:1.0 to about 1.7:1.0; (iii) a concentration of nitrate ions in the range from about 10 to about 26 mM/L is present; and (iv) a concentration of halide ions in the range from about 0.15 to about 4.0 mM/L is present.

17. A process according to claim 15, wherein: (i) the precursor mixture contains from about 0.380 to about 0.42 M/kg of H<sub>2</sub>TiF<sub>6</sub>; (ii) the ratio of total moles of component (A) to total moles of component (B) is in the range from 0.80:1.0 to 0.90:1.0; and (iii) the ratio of moles of silicon to moles of zirconium is in the range from 1.75:1.0 to 2.1:1.0.

18. A liquid metal treating composition made by a process according to claim 17, wherein: (i) titanium derived from component (A) of the precursor mixture is present in a total concentration from about 18 to about 25 mM/L; (ii) hexavalent chromium is present in an amount having a molar ratio to titanium, silicon, and zirconium atoms derived from components (A) and (B) in the range from about 1.10:1.0 to about 1.30:1.0; (iii) a concentration of nitrate ions in the range from about 14 to about 21 mM/L is present; and (iv) a concentration of chloride ions in the range from about 0.40 to about 0.80 mM/L is present.

19. A process for forming a corrosion protective coating layer on a metal surface, said process comprising steps of:

(IV) contacting the metal surface with a liquid metal treating composition according to claim 18 at a temperature in the range from about 21° to about 29° C. for a time in the range from about 75 to about 300 seconds;

(V) removing the metal surface from contact with said liquid metal treatment composition;

(VI) rinsing said metal surface with water; and, optionally, one or both of:

(VII) rinsing the metal surface after step (VI) with an aqueous composition comprising polymers of one or more  $x$ -(N—R<sup>1</sup>—N—R<sup>2</sup>-aminomethyl)-4-hydroxystyrenes, where  $x=2, 4, 5$ , or  $6$ , R<sup>1</sup> represents an alkyl group containing from 1 to 4 carbon atoms and R<sup>2</sup> represents a substituent group conforming to the general formula H(CHOH)<sub>n</sub>CH<sub>2</sub>—, where n is an integer from 1 to 7; and

(VIII) drying the rinsed metal surface.

\* \* \* \* \*